

# UNITED STATES PATENT OFFICE.

WALTER DYER AND WALTER EATON DYER, OF PORTLAND, OREGON.

## THINNED PAINT AND PROCESS OF MAKING PAINT-THINNER.

1,256,537.

Specification of Letters Patent. Patented Feb. 19, 1918.

No Drawing.

Application filed June 7, 1917. Serial No. 173,401.

To all whom it may concern:

Be it known that we, WALTER DYER and WALTER EATON DYER, subjects of the King of England, residing at Portland, in the 5 county of Multnomah and State of Oregon, have invented certain new and useful Improvements in Thinned Paint and Processes of Making Paint-Thinner; and we do declare the following to be a full, clear, and exact 10 description of the invention, such as will enable others skilled in the art to which it applies to make and use the same.

The present invention relates to the treatment of oils, particularly petroleum distillates consisting wholly or largely of paraffin hydrocarbons, such as ordinary kerosene, for use as a thinner or turpentine substitute, in mixed paints.

The process employed consists essentially 20 in adding alcohol, for example grain alcohol, denatured alcohol or wood alcohol, to the kerosene or similar oil, the amount of the alcohol being equal to about 5 to 10% by volume, relative to the amount of the oil; the 25 mixture is then heated to the boiling point, and the boiling is continued for a period of about half hour. The time of boiling is not absolutely fixed, but may be varied more or less, depending upon the proportions of the 30 ingredients, the gravity and other properties of the oil and other conditions. The material which is vaporized during the boiling operation may be led to a condenser coil and recovered if desired.

The oil thus treated is used as a thinner in 35 paints, for example by adding the same to a mixed paint consisting of linseed oil or vegetable oil treated in accordance with the process of our copending application Serial 40 No. 161,525, filed April 12, 1917. The turpentine substitute prepared as above described may also be added to paint oils generally as a thinner, for subsequent use in the same manner as mixtures of linseed oil and 45 turpentine are employed. The mixtures of the oil as above treated, with ordinary drying oils or the drying oils produced in accordance with our copending application above described, or the oil produced in accordance 50 with the process of Serial No. 130,038, filed November 7, 1916, are found to dry more quickly than without the addition of the turpentine substitute produced in accordance with the present process. The par-

affin oil produced in accordance with this process is also found to possess advantages over turpentine or benzine, not only in the point of cost, but that they have more body or density, than either turpentine or benzine or kerosene, and the petroleum oils treated 60 in the above manner may be directly mixed with pigments for the production of a thin drying paint.

We do not confine ourselves to the use of kerosene consisting entirely of paraffin hydrocarbons, since other grades of kerosene, particularly that produced from mineral oil of an asphaltic or semi-asphaltic base can be employed, or other oil distillates, the gravity of which may be somewhat above or somewhat below that of ordinary kerosene, with corresponding differences in the boiling point range.

The kerosene used may previously be refined if desired, although for many purposes 75 this is not necessary, and a crude kerosene can be employed, thereby saving the expense of the refining operation.

What we claim is:

1. A process which comprises adding to a 80 relatively larger bulk of a mineral oil distillate having a gravity about that of ordinary kerosene, a relatively smaller bulk of alcohol, and thereafter boiling the mixture, until drying properties are developed in the 85 oil.

2. A process of making a paint thinner, which comprises boiling a mixture of about 9 to 19 volumes of kerosene distillate with one volume of alcohol, for a period of about 90 half an hour.

3. A paint including as a constituent thereof, a paint thinner produced from kerosene by boiling with alcohol, said paint thinner having more body than kerosene, 95 gasoline or turpentine, and possessing drying properties, and being capable of hastening the drying of paints containing drying oils.

In testimony whereof we have hereunto 100 set our hands in the presence of two subscribing witnesses.

WALTER DYER.

WALTER EATON DYER.

Witnesses:

H. L. House,

Everett A. Johnson.